

## UNITED STATES PATENT OFFICE

2,451,270

## PRINTING WITH VAT COLORS

Chester Albert Amick and Roy Herman Kienle,  
Bound Brook, N. J., assignors to American  
Cyanamid Company, New York, N. Y., a cor-  
poration of Maine

No Drawing. Application July 31, 1944,  
Serial No. 547,512

6 Claims. (Cl. 8—70)

**1**  
This invention relates to new color compositions, to printing pastes prepared for use in printing on textile fabrics, paper and the like and to products printed therewith.

Use of printing-color pastes containing dyes, particularly in printing operations using vat dyes, is sufficiently well-known so that the procedure has become almost standardized. The actual color source may be either a dye paste or a dye powder. In addition to the real color, a dye paste usually contains agents to prevent drying-out, settling and/or freezing. Dye powders, not being subject to these difficulties, do not require these agents but they usually contain agents or are so processed as to promote dispersibility.

In either case, the dye paste or dye powder must be admixed with suitable thickener, usually a gum dispersion, to form a printing-color paste which is suitable for application. In the case of vat dyes, it is also necessary to add a reducing agent and usually an alkali. Because the color yield from a printing-color paste often decreases rapidly and the paste usually become too stiff for use as the paste ages after being made up, they are ordinarily prepared by the fabric finishers just before they are to be used.

However compounded, the printing-color pastes are then applied to textile, paper or other fabric materials for decorative or protective purposes. Subsequently, the printed pieces are dried, aged in a steam ager, treated with an oxidizing agent, rinsed and finally dried. Usually in processing textiles, the printed fabric also is soaped at or near the boil with about a 0.1% soap solution and again rinsed before the final drying operation.

In making up and applying printing-color pastes it has been found that a material suitable for use as a printing assistant is of advantage in obtaining maximum color yield. The exact way in which these materials act to produce an improved color yield in printing is not entirely understood. It is with color compositions containing such printing aids or assistants that the present invention is particularly concerned.

Although printing aids are desirable in the printing-color pastes, the exact point at which they are added may vary. Dye pastes may contain printing aids as one of their components and printing-color pastes made therefrom will obviously contain the printing assistant. Where a printing assistant is not present in the dye paste, it may be added at the time of making up the printing-color paste.

It is preferable, however, that the printing assistant be incorporated in the actual dye paste.

**2**  
Their addition at the proper point in the manufacture of the paste is not only easier, but in addition they are thus generally more uniformly dispersed throughout a printing-color paste made therefrom. As a result, the printing assistants usually operate more effectively when the printing-color paste is finally applied to the fabric.

It is only relatively recently that dye powders suitable for use in making up printing-color pastes have been available. Most of the printing aids previously used in dye pastes, being either liquid in form or extremely hygroscopic, can not be used with dye powders, the latter being necessarily limited to the use of dry solids. Nevertheless, it is desirable that printing assistants be incorporated in the powders at the time of manufacture for the same reasons which apply in the case of dye pastes.

**20** 20 Dye pastes containing various liquid printing assistants have been made. Among the liquid materials used are the alkylol amines, for example, triethanol amine; and/or polyhydric alcohols such as glycerine, glycol, diethyleneglycol and the like. Various derivatives therefrom also have been tried. When a printing aid is to be incorporated in a dye powder, a solid is necessary. Examples of such solids which have been used in the past include the hydrochlorides of alkylol amines; silver salt (sodium anthraquinone beta-sulfonate); anthraquinone and certain metal salts such as those of cobalt and iron.

Unfortunately, most of these printing aids previously used are not as satisfactory as may be desired. Many of them will not in all cases produce the intensification of color for which they were intended. Others, such as polyhydric alcohols, cause deterioration of the printing-color pastes so that marked variations in the strength of prints therefrom are observable even after the printing-color paste has been allowed to stand for only a relatively short time. Many of them are satisfactory with some colors but have an adverse effect on others, even to the extent of visibly altering the shade. None of them are suitable without modification for use both in paste and powder compositions.

There remains, therefore, a demand for suitable color compositions which will produce a satisfactory coloration when made into printing pastes and printed on the material but which are not subject to difficulties from deterioration or setting of the composition on standing. Preferably also, the color composition should be capable of derivation from either dye pastes or dye pow-

ders and the printing assistants used should therefore be obtainable in dry powdered form. In addition, they should be readily available or cheaply and easily prepared. Therefore, the principal objects of the present invention are to find suitable printing assistants and to combine them into color compositions and printing pastes.

In general these objects are accomplished by using as printing assistants the combination of urea or a substituted urea and a monoquinonyl amide of a dicarboxylic acid represented by the general formula



in which Q represents a quinonyl radical, Ac represents the residue of a cyclic or aliphatic dicarboxylic acid, and X represents hydrogen or an alkali metal radical.

So far as the present invention is concerned, the assistants may be added to the printing-color pastes in any of several ways during the compounding of the latter. They may be incorporated into the thickener; into the dye pastes or dye powders or they may be blended directly into the printing-color paste. However, as pointed out above, it is preferable that they be incorporated in the dye paste or powder during manufacture.

Use of these materials in the color compositions of the present invention has a number of advantages. Both of the compounds used are dry solids. Both are either soluble or dispersible in dye-paste suspensions. They have, therefore, a general application since they may be incorporated into either dye pastes or dye powders. They do not cause deterioration of printing-color pastes on standing. They tend to prevent setting up of the printing paste. They encourage the production of excellent color yields, even under hot ageing conditions. Their use is simple since they may be employed as either powders or as suspensions in water or alcohol, producing excellent color yields whatever the mode of admixture.

In preparing the amides to be used in the present invention, the dicarboxylic acid from which they are derived may be quite varied. Suitable acids include both cyclic and/or aliphatic dicarboxylic acids. Of the cyclic dicarboxylic acids, phthalic acid is perhaps the most common and its derivatives have been found to give good results when used according to the present process. The invention however is not meant to be so limited but includes derivatives of such acids as isophthalic, terephthalic, polyhydrophthalic, endoalkylene-polycydrophtalic acids such as endomethylene-tetrahydrophthalic and endoethylene-hexahydrophthalic acids and the like, and the naphthalic acids as well as substituted acids derived therefrom.

Where the derivatives of aliphatic dicarboxylic acids are used, the original acid or anhydride may be varied over a considerable range. If the original aliphatic acid is considered to have the generic formula



in the case of the anhydride, y may have substantially any value from zero, as in oxalic acid, to about eight. However, where y is greater than about six, difficulties are encountered in preparing the derivatives. Above about y=8, there is a tendency for the compounds to be too insoluble

for satisfactory use. The acids may be either saturated acids such as malonic, succinic, glutaric, adipic, azelaic, sebacic, and the like or unsaturated acids such as maleic, fumaric, and the like.

As pointed out in connection with the generic formula, Q represents a quinonyl group. Ordinarily however, Q will be limited to the beta-naphthoquinonyl and the alpha and beta anthraquinonyl radical. Alpha-naphthoquinone appears to transform to the beta derivative in forming the amide. The invention however is not necessarily so limited since quinonyl radicals having various substituents on the ring may be used.

The exact function of the urea or substituted urea and its mode of operation is not fully understood. There is a possibility that there is an association between it and the monoquinonyl amide which breaks down under conditions of use as well as that the two remain separate entities. In any case, however, the result obtained is far superior to that obtained by the use of either alone, or would be expected from the use of either alone.

Urea itself, being the most readily available of the ureas is probably preferable for use in the compositions of the present invention. Particularly is this true since it produces wholly satisfactory color yields and its other physical properties are satisfactory. The invention, however, is not limited thereto. Substituted ureas, particularly the alkyl and alkylol ureas in which the substituent group contains up to about six carbon atoms, phenyl urea, guanyl urea and dicyanamide may be used effectively if so desired.

In using urea, or substituted ureas, it is often preferable to colloidize the urea for ease in handling and it insures thorough dissemination. This is quite simply carried out by thoroughly mixing one part of urea and about three parts of dextrin, preferably yellow corn dextrin with a small amount of water in a Banbury mixer or the like. The resultant product is then vacuum dried at about 60°-70° C. and ground to about minus 140 mesh. When colloidized in this manner, the urea is particularly well adapted for use in powder compositions.

While the dye and printing paste compositions of the present invention are not limited to the use of any particular dyes or dye forms, they are especially suitable for use with vat-dyes in either paste or powder form. Particularly good results may be obtained using vat-dye powders of high auto-dispersibility as set forth in Crossley et al., United States Reissue Patent 21,402, reissued March 19, 1940. By combining the color materials of that patent into the compositions of the present invention, the full advantages of both may be gained with a resultant simplicity in use and excellence of shade and sharpness of color.

Printing pastes made in this way have the particular advantage that the dyes remain in a highly dispersed state as individual particles rather than as dispersions of particle aggregates. In the present specification and claims, where highly-dispersed dyes are referred to, reference to pastes in which the dye particles are so dispersed is intended.

The invention will be more fully set forth in connection with the following examples which are intended to be illustrative and not by way of limitation. All parts are by weight unless otherwise noted.

In the succeeding examples, test prints were made on two different types of fabrics. When rayon is referred to, a titanium-dioxide-pig-

mented, all-viscose rayon flat crepe was used. The cotton fabric referred to is an 80 x 80 bleached, unmercerized, cotton print-cloth. Ageing of the prints was carried out in a steam ager which was constructed in such a manner that controlled temperatures could be used. The temperature range normally used was 100°-105° C. Those ageings referred to as plant or hot ageings were carried out in the temperature range of about 106°-110° C. In the case of the cotton prints ageing periods of 3 minutes, 5 minutes or both were used. On rayon, ageing periods of 5 to 10 minutes or both were used. The shortest period which gives a satisfactory ageing is preferable.

*Example 1*

A paste was prepared by slurring 2,000 parts of 177 British gum (Stein Hall) in 5,000 parts of water and the mixture was heated with continuous stirring until the temperature reached about 185° C. Heating was continued for about 1½ hours after which 450 parts of powdered sodium carbonate and 450 parts of powdered potassium carbonate were added and the mixture stirred until the carbonates dissolved. Heating was discontinued but stirring was continued until the temperature reached approximately 150° F. at which time 700 parts of sodium sulfoxylate formaldehyde were dissolved therein. Subsequently, 600 parts of glycerine were added and the paste bulked to about 10,000 parts. Stirring was continued until the paste cooled to room temperature. In the succeeding examples this paste is referred to as thickener A.

*Example 2*

720 parts of B-2 British gum and 720 parts of KAC-4 gum (Stein Hell) were added to 5,600 parts of water and heated over a steam bath for approximately 1½ hours after the temperature reached 185°-190° F. The source of heat was then removed but stirring was continued until the temperature decreased to 120° F. at which time 1,200 parts of potassium carbonate which had been previously dissolved in 1,000 parts of water was added to the cooked gum. 1,560 parts of sodium sulfoxylate formaldehyde were dissolved in 1,500 parts of water at a temperature of about 140° F. and added to the common mixture with stirring until the whole was thoroughly mixed. 360 parts of glycerine were then added and after thorough stirring the whole was bulked to 12,000 parts. In the succeeding examples this mixture is referred to as thickener B.

*Example 3*

48 parts of Orange R (Color Index 1217) presscake containing 12 parts real color were diluted with 52 parts of water to make a uniform suspension. 10 parts of this color suspension, 5 parts of a 6% slurry of the alpha-anthraquinonyl mono amide of maleic acid and 5 parts of water were intimately mixed, after which 80 parts of thickener A were added. This printing color paste was used as the control. To a second 10 parts of the Orange R slurry were added 5 parts of a 6% suspension of the alpha-anthraquinonyl mono amide of maleic acid and 5 parts of urea, after which 80 parts of thickener A were added.

Both color pastes were then printed on pigmented ( $TiO_2$ ) viscose rayon and on 80 x 80 bleached, unmercerized cotton print cloth, dried in a hot air dryer at a low temperature, aged in a steam ager, treated with an oxidizing agent, rinsed, soaped in a 0.1% soap solution for 5

minutes at the boil, again rinsed, and ironed dry.

Prints made from the paste containing the urea are stronger and brighter than the prints made from the prints made from the paste in which no urea was used.

*Example 4*

The procedure of Example 3 was repeated exactly, except that a 6% suspension of the beta-anthraquinonyl monoamide of maleic acid was used in place of the alpha-anthraquinonyl monoamide. Prints made from the paste containing urea and the beta-anthraquinonyl mono-amide of the maleic acid were bright and appreciably stronger than those made from the paste containing no urea.

*Example 5*

The procedure of Example 3 was again repeated exactly except that the beta-anthraquinonyl monoamide of phthalic acid was used in place of the beta-anthraquinonyl monoamide of maleic acid. Bright, strong prints are obtained when the urea was used, and the ageing is carried out at a temperature of about 108° C. These prints are stronger than those obtained when no urea is used.

*Example 6*

The procedure of Example 3 was repeated except that the alpha-anthraquinonyl monoamide of succinic acid was used in place of the alpha-anthraquinonyl monoamide of maleic acid. The results were essentially those obtained in Example 3 being better than when no urea is used.

*Example 7*

The procedure of Example 3 was repeated except that the alpha-anthraquinonyl monoamide of fumaric acid was used instead of the alpha-anthraquinonyl monoamide of maleic acid. Again the addition of urea caused improved results to be obtained.

*Example 8*

Again the procedure of Example 3 was repeated except that the alpha-anthraquinonyl monoamide of maleic acid was replaced by the beta-naphthoquinonyl monoamide of maleic acid. Substantially duplicate prints of those of Example 3 were obtained.

*Example 9*

A Vat Yellow GC presscake (Color Index 1118) was slurred with water to give about a 10.5% suspension. The procedure of Example 3 was repeated exactly using the Yellow GC color instead of the Orange R. The print from the paste in which the urea was present was stronger and fuller than the print obtained from the paste in which no urea was used, particularly in commercial-type ageing.

*Example 10*

The procedure of the preceding experiment was repeated exactly except that thickener B was substituted for thickener A. The results were essentially the same, the paste containing urea giving a stronger and fuller color value than the paste in which no urea is present.

*Example 11*

The procedure of the preceding Example 9 was repeated exactly except that 10 parts of a Vat Navy Blue aqueous dispersion (Color Index 1100) containing about 1.8 parts of real color is used in place of the Vat Yellow GC. The prints made

from the paste containing the urea were stronger and brighter than those made from the paste in which no urea was present.

*Example 12*

3 parts of a dispersible Orange R powder (Color Index 1217) prepared according to U. S. Reissue Patent 21,402 and containing about 1.2 parts of real color, were dry blended with 0.3 part of the alpha-anthraquinonyl monoamide of maleic acid. 10 11.7 parts of water were added to this and intimately mixed. 85 parts of thickener B were added and after mixing to form a smooth paste, was used as the control sample. A second printing paste was prepared by using 3 parts of the same color, and dry blending therewith 0.3 part of the alpha-anthraquinonyl monoamide of maleic acid and 5 parts of urea. To this was 15 20 added 8.7 parts of water and after thorough mixing 85 parts of thickener B were added thereto. These color pastes are then printed and finished as in Example 3. Prints made from the paste in which both the alpha-anthraquinonyl monoamide of maleic acid and urea were present were definitely stronger and brighter than those obtained 25 from the pastes in which no urea was used.

*Example 13*

Again the procedure of Example 12 was repeated except that 20 parts of colloidized urea (prepared from urea and dextrin is a 1:3 ratio) were substituted for the 5 parts of urea. The dry blending operation was more easily carried out. Prints obtained from both the control sample and that containing the colloidized urea were substantially the same as those of Example 11 although on the rayon sample the color yield was slightly improved by using colloidized urea.

We claim:

1. A color composition comprising essentially a vat-dye, a quinonyl monoamide of a dicarboxylic acid, the quinonyl radical being selected from the group consisting of the beta-naphthaquinonyl and alpha- and beta-anthraquinonyl radicals, and a urea.
2. A dye powder composition comprising essentially a dry vat-dye powder, a dry, powdered quinonyl monoamide of a dicarboxylic acid, the quinonyl radical being selected from the group consisting of the beta-naphthaquinonyl and alpha- and beta-anthraquinonyl radicals, and a dry powdered urea.

3. A dye powder composition comprising essentially a dry vat-dye powder of high auto-dispersibility, a dry powdered quinonyl monoamide of a dicarboxylic acid, the quinonyl radical being selected from the group consisting of the beta-naphthaquinonyl and alpha- and beta-anthraquinonyl radicals, and a dry powdered urea.

4. A dye powder composition comprising essentially a dry vat-dye powder of high auto-dispersibility, a dry powdered quinonyl monoamide of a dicarboxylic acid, the quinonyl radical being selected from the group consisting of the beta-naphthaquinonyl and alpha- and beta-anthraquinonyl radicals, and a dry powdered urea colloidized with dextrin in the ratio of about 1:3.

5. A printing-paste composition comprising essentially a thickener, a vat-dye, a quinonyl monoamide of a dicarboxylic acid, the quinonyl radical being selected from the group consisting of the beta-naphthaquinonyl and alpha- and beta-anthraquinonyl radicals, and a urea.

6. A method of printing with vat color which comprises printing with a printing paste composition comprising essentially a thickener, a vat-dye, a quinonyl monoamide of a dicarboxylic acid, the quinonyl radical being selected from the group consisting of the beta-naphthaquinonyl and alpha- and beta-anthraquinonyl radicals, and a urea.

CHESTER ALBERT AMICK,  
ROY HERMAN KIENLE.

REFERENCES CITED

The following references are of record in the file of this patent:

UNITED STATES PATENTS

| Number       | Name       | Date          |
|--------------|------------|---------------|
| 1,963,967    | Berthold   | June 26, 1934 |
| 1,970,644    | Berthold   | Aug. 21, 1934 |
| 2,004,458    | Berthold   | June 11, 1935 |
| 2,063,147    | Berthold   | Dec. 8, 1936  |
| 2,090,511    | Crossley   | Aug. 17, 1937 |
| 2,128,599    | Albrecht   | Aug. 30, 1938 |
| 45 2,145,193 | Kern       | Jan. 24, 1939 |
| 2,184,495    | Graenacher | Dec. 26, 1939 |
| 2,196,958    | Crossley   | Apr. 9, 1940  |
| 2,233,101    | Kern       | Feb. 25, 1941 |
| 2,286,262    | Clark      | June 16, 1942 |